

## UNITED STATES PATENT OFFICE.

ROYER LUCKENBACH, OF BROOKLYN, NEW YORK, ASSIGNOR TO LUCKENBACH PROCESSES, INC., OF SAN FRANCISCO, CALIFORNIA, A CORPORATION OF NEVADA.

## CONCENTRATION OF ORES BY FLOTATION.

No Drawing.

Application filed March 6, 1920. Serial No. 363,865.

*To all whom it may concern:*

Be it known that I, ROYER LUCKENBACH, a citizen of the United States, and a resident of the borough of Brooklyn, county of 5 Kings, city and State of New York, have invented a certain new and useful Concentration of Ores by Flotation, of which the following is a specification.

The invention relates to the concentration 10 of ores by flotation and has for its objects to use a cheap and effective reagent which will not only attract and be attracted by the mineral values in the pulp, but will also form a copious froth of great dryness capable of supporting and floating a relatively 15 large amount of mineral particles, but will reject the earthy or gangue particles, whereby a clean concentrate may be formed.

A further object is to use a reagent of 20 which such an infinitesimal amount is employed that its presence in the concentrate will not materially affect subsequent steps in the recovery and manufacture of the values, and which is itself of such little value, that 25 its recovery need not be attempted.

These and further objects will more fully appear in the following specification and claims.

In the flotation process of ore concentration as at present carried out, coal tar, and 30 coal tar creosote are largely employed as gathering agents. Such substances are not freely miscible in water, and in order to be of any effect in the flotation machine they 35 must first be beaten into the pulp, or the water of the pulp, by vigorous agitation in order to break the tar or creosote up into globules which will enter into the pulp in the flotation machine and form the emulsion. 40 so called, which apparently is necessary in the carrying out of the oil flotation process.

By means of the present invention, coal tar, coal tar creosote, wood tar and wood tar creosote are formed into a colloid solution, 45 and may be placed in the flotation machine without further treatment, and will produce in the pulp a perfect emulsion.

In carrying out the preferred embodiment 50 of the invention coal tar, or coal tar creosote is mixed with a soluble ketone and the mixture is dissolved in a solution of an alkali in water.

The ketone employed may be acetone, and it may be used alone or it may be mixed with 55 alcohol (ethyl, methyl, or denatured), or

carbon di sulphide may be used as the tar or creosote solvent.

The preferred alkali for use in the mixture is caustic soda, but other alkalies, or carbonate of soda, may be used.

If desired the reagent may be acidified by adding an acid, such for example as sulphuric acid, to the reagent until the alkali is neutralized. This acidified reagent is particularly adapted for use with ores of an acid 65 nature.

In the preferred embodiment of the invention, 10 cc. of coal tar, or coal tar creosote, and 5 cc. of ethyl acetate are mixed in warm water with stirring. This forms a more or 70 less syrupy liquid which is preferably diluted with 180 cc. of warm water. This is the reagent. The temperature of the water should be less than the boiling point.

Instead of employing coal tar or coal 75 tar creosote as above, a mixture of 5 cc. of coal tar and 5 cc. of creosote may be used. The combined coal tar and creosote mixture is preferred as such mixture emulsifies better than either alone.

In carrying out the process approximately 8 cc. of the reagent is employed per 1 gallon of water in the pulp. The reagent is miscible in the water, and will immediately 80 spread throughout the pulp.

In a test 500 grams of a New Mexican chalcopyrite copper ore was treated in a Janney flotation machine, with 8 cc. of the reagent in 1 gallon of water.

The ore assayed 4.04% copper.

The machine was run for 4 minutes and a thick, dry, fine grain froth was removed from the surface of the pulp. The concentrate of this froth weighed 65.9 grams and assayed 15.15% copper.

A further run of 3 minutes was made and another froth produced. The middlings, solid content of this second froth weighed 140.3 grams, and assayed 6.62% copper.

The tailings weighed 291.5 grams and assayed 0.33% copper.

The extraction shown in the test was 94.4% of the copper content of the ore.

The creosote, or other active substance which is comprised in the reagent is, by 105 reason of the reaction with the ketone and the alkali, reduced to extremely fine particles each of which is capable of attracting, or being attracted by, the mineral values in the pulp, and will form, or be incorporated 110

in, the films of the bubbles by the aeration of the pulp, and will rise to the surface bearing, the mineral particle or particles adhering thereto and form a thick, tenacious and fine 5 grained froth on the surface of the pulp.

The proportions above given are approximate only. Some ores, or some runs of the same ore, may require a stronger reagent than others. With some ores the tar or 10 creosote may be greater in proportion to the ketone, or the alkali content may be strengthened or weakened.

Coal tar and coal tar creosote are largely employed in oil flotation processes. These 15 substances are not naturally miscible in water, or at the most are only partially so. When used they must be violently beaten into the water to break the oil up into globules, and the agitation must be continued 20 in the pulp to keep the globules in suspension and prevent them floating to the surface and coalescing into a film. The coal tar and creosote as commonly used in the oil flotation process are indifferent frothers and 25 are usually supplemented by a frothing oil, and a frothing oil, such as used in flotation is an expensive commodity.

By the invention of this application the gathering or collecting properties of the tar 30 and creosote are greatly increased, and the mixture possesses the added property of producing a copious froth, which will be clean. As will be seen in the example given above the reagent is composed very largely of 35 water, and the proportion of the other materials entering into its composition are almost infinitesimal in comparison to the water and ore in the pulp.

If desired the reagent may be compounded 40 in greatly condensed form by reducing the water content. This will provide for cheap transportation. In use, however, it will, because of the minuteness of the quantity of the active materials used in the pulp, be 45 possible to dilute the mixture whereby rough measurement as to the quantity to be used, may be made.

It is to be understood that instead of coal tar, or wood tar or their creosotes, shale tar 50 and some, at least, of its derivatives may be

employed, and that in this specification and claims the term "oily distillate" is intended to mean any of them. It is further to be understood that while the "distillates" above mentioned are normally oils, or of an oily nature, they have nothing of an oily nature when reduced and neutralized as above described, and that there is no free oil used in carrying out the process of the application.

In accordance with the provisions of the patent statutes the principle of the invention, has been described together with the process which is now considered to represent the best embodiment thereof, but it is understood that the process described is merely 65 illustrative, and that the invention may be carried out in other ways.

Having now described the invention what is claimed and desired to be secured by Letters Patent of the United States, is—

1. The process of concentrating ore, which comprises mixing the ore with water to form a pulp, introducing a reagent comprising the reaction product of coal tar and coal tar 75 creosote and a ketone and caustic soda into the pulp, aerating the pulp to form a froth, and removing the froth from the pulp.

2. The process of concentrating ore, which comprises mixing the ore with water to form a pulp, introducing a reagent comprising an acidified reaction product of coal tar and coal tar creosote and a ketone and caustic soda into the pulp, aerating the pulp to form a 80 froth, and removing the froth from the pulp.

3. The process of concentrating ore which consists in mixing the ore with water to form a pulp, introducing a reagent comprising the reaction product of coal tar and coal tar 85 creosote and a ketone, mixed with a solution of an alkali in water, aerating the pulp to form a froth, and removing the froth from the pulp.

This specification signed and witnessed 90 this fourth day of March, 1920.

ROYER LUCKENBACH.

Witnesses:

J. F. COLEMAN,  
A. E. RENTON.